

Sept. 23, 1924.

1,509,353

C. C. HALL

PACKING

Filed Jan. 11, 1924



FIG. I.



FIG. II.



FIG. IV.



FIG. III.



FIG. V.

INVENTOR  
Charles C. Hall  
BY  
Chappell Dear  
ATTORNEYS

## UNITED STATES PATENT OFFICE.

CHARLES C. HALL, OF KALAMAZOO, MICHIGAN.

## PACKING.

Application filed January 11, 1924. Serial No. 685,566.

*To all whom it may concern:*

Be it known that I, CHARLES C. HALL, a citizen of the United States, residing at the city and county of Kalamazoo, State of Michigan, have invented certain new and useful Improvements in Packings, of which the following is a specification.

This invention relates to improvements in packings.

10 The main object of this invention is to provide an improved packing which is well adapted for general use on steam or hydraulic packings and for high temperatures and heavy pressures.

15 A further object is to provide an improved packing which is strong and durable and at the same time has good anti-friction and lubricating qualities.

Further objects, and objects relating to 20 structural details, will definitely appear from the detailed description to follow.

I accomplish the objects of my invention by the devices and means described in the following specification. The invention is 25 clearly defined and pointed out in the claims.

A structure which is a preferred embodiment of my invention is clearly illustrated in the accompanying drawing, forming a part of this application, in which:

30 Fig. I is a fragmentary plan view of a thin sheet of metal or metal foil such as I employ in my improved packing.

Fig. II is a plan view of the sheet crumpled and coated with lubricant.

35 Fig. III is a detail view illustrating one of the steps of manufacture, the thickness of the metal being very greatly exaggerated for convenience in illustration.

Fig. IV is a cross section through my 40 improved packing in cylindrical cross section, the lead and the aluminum being indicated by the difference in cross sectioning.

Fig. V is a detail perspective view of my 45 improved packing reduced to rectangular cross section.

In the drawing similar reference characters refer to similar parts throughout the several views.

Referring to the drawings, 1 represents a 50 thin sheet of metal or metal foil such as I employ in my improved packing and 2 is a

sheet crumpled and coated with lubricant, preferably a paste or powdered flake graphite and high temperature oil, although beeswax, japan wax, glycerine or other lubricant 55 may be employed.

I employ one or more sheets of the aluminum foil indicated at 3 and one or more sheets of lead foil indicated at 4. These thin sheets of aluminum and lead foil are both 60 coated with the lubricant and crumpled and then wound together preferably with the aluminum at the outside.

The lubricant is retained between the 65 sheets and in the pockets thereof so that it is in quite uniformly distributed condition and in sufficient quantities to form a self-lubricating packing, the lead itself being regarded by some authorities as an effective lubricant.

70 The aluminum foil is preferably 1/1000 of an inch in thickness and is preferably annealed. The lead foil is also thin but may be considerably thicker than the aluminum foil with satisfactory results.

75 My improved packing may be left in the cylindrical form as indicated in Fig. IV or it may be compacted into a rectangular form as shown in Fig. V.

80 My improved packing is desirable for many uses, it being highly desirable for instance in saturated steam up to 160 pounds pressure or for hydraulic packings, particularly high pressures, and in various relations where lead has been deemed a desirable 85 packing. It does not, however, have the objection that is found in lead packings of solidifying under high temperatures and pressures, the aluminum being incorporated throughout with the lead enabling the packing to be used under such temperatures and pressures as would render a packing of lead impracticable. Further, it has greater 90 strength.

95 My improved packing is also highly desirable for parts moving at high speed, for instance, centrifugal pumps and the like.

Having thus described my invention, what I claim as new and desire to secure by Letters Patent, is:

1. A packing comprising a sheet of aluminum and a sheet of lead crumpled, coated

with lubricant, superimposed and rolled together so that the aluminum is at the outside, and compacted.

2. A packing comprising a sheet of aluminum and a sheet of lead, coated with lubricant, superimposed and rolled together so that the aluminum is at the outside.

3. A packing comprising a sheet of aluminum and a sheet of lead crumpled, coated with lubricant and rolled together.

In witness whereof, I have hereunto set my hand.

CHARLES C. HALL. [L. S.]